

# UNITED STATES PATENT OFFICE.

ALEXANDER H. SIEGFRIED, OF SELIN'S GROVE, PENNSYLVANIA.

## COMPOUND FOR TEMPERING STEEL.

SPECIFICATION forming part of Letters Patent No. 257,248, dated May 2, 1882.

Application filed September 24, 1881. (No specimens.)

*To all whom it may concern:*

Be it known that I, ALEXANDER H. SIEGFRIED, of Selin's Grove, in the county of Snyder and State of Pennsylvania, have invented 5 certain Improvements in Compounds for Tempering Steel, of which the following is a specification.

My invention relates to an improved compound for use in preparing and tempering steel.

10 In making use of my invention I first prepare a compound consisting of salt, four and a half pounds; sulphate of copper, three-fourths of a pound; soda-ash, one and one-half pound; sal-ammoniac, one pound; oxide of manganese, three-fourths of a pound; sulphate of iron, three-fourths of a pound; nitrate of potassa, one-half of a pound. These ingredients are pulverized and thoroughly intermingled to produce a homogeneous mass. The steel to be 15 treated is heated to a red heat and the compound applied thereto, after which the steel is returned to the fire and heated to a proper degree for working, then withdrawn and worked on the anvil into the required shape. This 20 operation is repeated until the tool is finished and ready for tempering, when it is heated to a cherry-red heat, the compound applied, and the tool subsequently tempered to give it the

desired degree of hardness in the usual way. I find that by means of the compound and the 30 treatment above described I am enabled to give the cutting-tool a great degree of hardness combined with great strength and toughness.

While it is preferred to adhere to the proportions stated, they may be modified to a limited extent without seriously affecting the action of the compound.

The heating of metal and the application of the compound thereto may be repeated any 35 40 desired number of times, steel which contains an excess of carbon requiring a more thorough application of the compound than the steels in which the percentage of carbon is smaller.

Having thus described my invention, what 45 I claim is—

The compound for tempering steel, consisting of salt, sulphate of copper, soda-ash, sal-ammoniac, oxide of manganese, sulphate of iron, and nitrate of potassa, in substantially the proportions specified.

ALEXANDER HIRAM SIEGFRIED.

Witnesses:

GEORGE EBY,  
VAL. BOLIG.